

1,102,332.

G. FLAWITH.  
LUBRICATING PACKING.  
APPLICATION FILED DEC. 23, 1912.

Patented July 7, 1914.



WITNESSES

A. T. Palmer  
Anna B. Lindsey

INVENTOR  
GEORGE FLAWITH  
BY  
Mitchell, Chasnick & Kurt  
ATTYS.

# UNITED STATES PATENT OFFICE.

GEORGE FLAWITH, OF MELROSE HIGHLANDS, MASSACHUSETTS.

## LUBRICATING-PACKING.

1,102,332.

Specification of Letters Patent.

Patented July 7, 1914.

Application filed December 23, 1912. Serial No. 738,281.

*To all whom it may concern:*

Be it known that I, GEORGE FLAWITH, a subject of the King of Great Britain, residing at Melrose Highlands, in the county of 5 Middlesex and State of Massachusetts, have invented new and useful Improvements in Lubricating-Packing, of which the following is a specification.

This invention relates to improvements in 10 lubricating packing.

More particularly it relates to a composition or article of manufacture for holding a supply of oil against a surface which requires lubrication, either loosely, as in the 15 axle box of a railroad car, or tightly, as in a gland packing for a piston rod under fluid pressure.

It is the object of the invention to provide an improvement upon compositions that 20 have been hitherto used or known for this purpose. Cotton waste which is commonly used by the railroads as being on the whole most satisfactory, requires relatively frequent attention. Failure to give such attention in proper season results in a "hot 25 box", occasions delay and interrupts the service.

It is one object of the invention to provide a composition which is practically free 30 from the requirement of such attention owing to the very long time through which it will maintain itself in good running condition. Efforts have been made to improve packing by using other substances in place 35 of cotton waste.

It is among the objects of the present invention to improve over them as well as over the cotton waste.

None of the compositions heretofore proposed, so far as I am aware, are automatically safeguarded for conditions when the oil content has become below normal; and all so far as I am aware, are wasteful of oil, in the sense that they absorb into their 45 own substance a substantial quantity of the oil and thus render unavailable oil which otherwise might be available for lubrication of the bearing surface.

It is a further object of the invention to 50 provide improvement in these two respects, viz., to provide a composition which can, if events so happen, run rather dry without disastrous effects, and one which holds a very high proportion of its oil available for 55 efficient use. Another difficulty in connection with the lubrication of bearings, par-

ticularly of axle bearings on cars, has been the tendency of the packing to settle away from the journal. Numerous efforts have been made to remedy this, but I am not 60 aware of anything that has done so in a commercial successful and satisfactory way prior to the invention herein set forth, notwithstanding the claims or expectations with which various products have been put forth 65 to the public; and it is a further object of the present invention to provide a composition that actually will not settle away when properly packed, and that can in practice be "properly" packed easily by ordinary workmen employing only ordinary skill and attention and working under ordinary service conditions.

It is also the object of the invention to attain the other advantages which characterize 75 the composition herein disclosed; and it is the object of the patent to cover in the claims such features of novelty as exist in the invention herein disclosed.

The main features of the improvement result from the use of a tough elastic filiform supporting material intermingled with suitable fibrilliform material; and it is a particular feature of the invention to make the former of partially dried animal entrails or 80 "gut." The other material may be finely shredded asbestos or leather, or other material. The advantage of asbestos is that it is light in weight, does not absorb oil, and is itself somewhat of a lubricant; while leather 85 is still lighter and has other advantages. When the mixture is complete the greater part of its is composed of this soft shredded fibrous material, with fibers but a fraction of an inch in length, which however is long enough so that they adhere to each other, 90 become somewhat entangled with each other, and have capillary and other spaces among them for the reception and holding of the oil or other lubricant. Running in all directions through this mass of soft material, and holding it up, is the elastic, rough surfaced filiform material first described above. This latter may be prepared by simply drying 95 the intestine of the sheep or other animal. When so prepared, this tubular intestinal tissue or fiber shrinks into small diameter, that which I have used with success being from sheep similar to that used for ordinary sausages, and being when dry about one-thirty-second of an inch or more in diameter; becomes irregular, both in thickness and 100 105 110

in cross section; hardens and stiffens with a rough surface; twists more or less; and acquires somewhat elastic, wiry characteristics, besides being naturally strong and tough. If the material be not tubular at the start it may be well to slit it into proper widths before it is very dry. It is also well to curl it somewhat in drying, as by winding around a rod, or allowing it freedom to shrink; and to stop the drying before it has become too brittle, and thus saving some of its own oil.

The asbestos, leather, or other fibrilliform material is prepared by any suitable grinding or shredding process. Then the two are thoroughly mixed. I will describe the method which I consider best in connection with leather, which is to mix the shredded leather with lubricating oil for a period of twenty minutes, or thereabout, then to let it stand for a day to become saturated, and then to put in about three pounds of the filiform material to one hundred pounds of the combined leather fibers and oil, although this proportion may be varied, and then to mix the whole. The filiform material may be in lengths of eight to ten inches. If the pieces have been curled in loose spirals they can hold the fibers better, because masses of fibers are embraced between their successive coils.

In the accompanying drawing, an embodiment of the invention is illustrated in use in connection with a car axle.

In the drawing, Figure 1 is a side elevation of the journal box of the car axle with the packing in place, in medial section; and Fig. 2 is an end elevation of the same, in section.

In the drawing, the car axle is marked 10. The journal, through which the weight of the car rests down upon the axle, is marked 11. The journal box is 12, having a door 13 through which the bearing may be inspected and packing inserted; and the packing itself consists of the fibrilliform material 14 and the filiform material 15, which is represented, somewhat arbitrarily, as being interwoven and intermingled in the mass of fibrilliform material, with the effect of holding such mass up in contact with the under side of the axle.

When desired for use a suitable quantity of the composition is placed in the axle box of a railroad car, for example. The composition should be packed up against the under sides and the end of the axle, so that it is well in contact therewith, as ordinary packing at present is commonly used. The main reliance for holding the oil is the minute interstices between the fibers. Practically all of the oil is available for lubricating purposes, when the fibrous material is asbestos combined with filiform gut as above described, because all the oil is on the surface

of the fibers. A saving of oil is therefore effected as compared with fibers of wool, leather or other materials which absorb an appreciable quantity of oil into their own substance. Inasmuch as both the asbestos and the gut are inherently lubricators, especially so as compared with leather or wool or hair or cotton, there is less likely to be harm to the bearing if it runs too dry, or if some of the material of the packing be drawn through. These materials, also, are not inclined to char, or carbonize as are materials heretofore used, if the bearing runs hot. When the oil is present the gut becomes soft and more slippery, but I have found in practice that, on the one hand, it retains sufficient stiffness and elasticity to hold the mass up against the moving surface of the axle; and yet, on the other hand, is not apt to be drawn under the brass bearing.

Having thus defined the invention it will be obvious that any suitable lubricating agent, such as oil or grease or the like, may be employed with the composition to form the complete lubricating packing, and that mica or graphite flakes may be used in this connection; also that fibrilliform material of different varieties may be combined in any desired proportions and used with the filiform support. When a bearing has once been properly packed with the composition of the invention it will run for a very long time without further attention, a particular effect of the tough elastic filiform gut components being that it keeps the composition from rolling into balls, or settling, or being worked away from the axle. It will be understood that the word "filiform" does not limit the element to which it refers to any particular size, but means that it is in the general form of a thread or filament as contrasted with the "fibrilliform" material, which term as here used signifies a material in which numerous small fibers have been separated from their natural proximity to each other to provide oil holding spaces between them and are gathered in a loose mass or masses.

When the invention is used in connection with the packing of glands for plungers, piston rods, etc., under steam, air, hydraulic or any other pressure, the composition described may be interwoven with any other substance, in order to make a stationary body, or it may be used as above described; and its component materials are such that it will resist both heat and moisture satisfactorily.

What I claim is:

1. A composition adapted for a lubricating packing, including, in combination, leather finely divided into fibrilliform condition and gut in filiform condition intermingled therewith.

2. A composition adapted for lubricating

125

110

100

95

90

85

80

75

70

65

60

55

50

45

40

35

30

25

20

15

10

5

packing, including, in combination, a mass of finely divided oil holding fibrilliform material and filiform cured intestinal tissue intermixed therewith and supporting the higher portions thereof.

3. The method of making a lubricating packing comprising the shredding of leather into finely divided fibrilliform condition; saturating it with lubricating oil; and mixing therewith filiform gut.

4. The method of making a lubricating packing comprising the curing separately of

animal hide and intestinal tissue; forming separately the hide into fibrilliform condition and the intestinal tissue into filiform <sup>15</sup> condition; and then saturating the fibrilliform material with a lubricant and mixing the filiform material through the mass.

Signed by me at Boston, Mass., this nineteenth day of December, 1912.

GEORGE FLAWITH.

Witnesses:

JOSEPH T. BRENNAN,  
EVERETT E. KENT.